

Jan. 16, 1951

P. H. CARNELL  
PROCESS FOR FLUOSULFONIC ACID  
REFINING OF LUBRICATING OIL  
Filed Dec. 15, 1947

2,538,293



INVENTOR.  
PAUL H. CARNELL

BY

*Hulson & Young*

ATTORNEYS

## UNITED STATES PATENT OFFICE

2,538,293

PROCESS FOR FLUOSULFONIC ACID  
REFINING OF LUBRICATING OILPaul H. Carnell, Alma, Mich., assignor to Phillips  
Petroleum Company, a corporation of Delaware

Application December 15, 1947, Serial No. 791,804

4 Claims. (Cl. 196—39)

1

This invention relates to the treatment of lubricating oils to improve their properties. In one of its more specific aspects it relates to treatment of a lubricating oil to improve its viscosity index.

I have discovered that treatment of a lubricating oil with fluosulfonic acid, and if desired, a low-boiling hydrocarbon, such as, iso- or normal pentane, will improve the viscosity index of the oil.

Lubricating oil referred to herein, includes all such products and their base stocks which have a viscosity within the range of about 32 SUS (Saybolt Universal seconds) at 210° F. to about 350 SUS at 210° F., and as are usually understood to be covered by this term by those skilled in the art. It includes lubricating oil stocks, such as, paraffin-base stock, naphthene-base stock, synthetic-base stock, and mixed-base stock, which are refined for use as engine lubricants.

The important improvement in oils treated by the present process is in the viscosity index which is determined by the method described in the article entitled "Viscosity Variations of Oils with Temperatures," by E. W. Dean and G. H. G. Davis, in Chemical and Metallurgical Engineering, volume 36, pp. 619 (1929). The viscosity index of a lubricating oil is an indication of its composition or type, i. e., whether it is a paraffin-base or naphthene-base oil. Paraffin-base oils have high viscosity indices, naphthene-base oils have relatively low viscosity indices, and mixed-base oils have viscosity indices between these two. This index is likewise a measure of the ability of a lubricating oil to remain viscous at high temperatures. As is well known, oils lose their viscosity rapidly with an increase in temperature. The oil with a high viscosity index will, however, lose its viscosity less rapidly than an oil with a low viscosity index when the temperature is increased, or conversely, will not have its viscosity unduly increased by a lowering of temperature. The present invention increases this viscosity index.

I have discovered that fluosulfonic acid ( $\text{HSO}_3\text{F}$ ) is an excellent refining agent for lubricating oils. Further, I have found that, under suitable reaction conditions, this acid is superior to hydrofluoric acid in producing high viscosity index oils. Also in the processing of certain lubricating oils, particularly mixed-base oils, fluosulfonic acid treating yields higher viscosity indices than treating with sulfuric acid under similar conditions.

An object of the present invention is to provide a method for improving lubricating oils. An-

other object is to provide a method for improving natural lubricating oils. A further object is to provide a method for improving synthetic lubricating oils. Another object is to provide a method for improving mixed-base lubricating oils. A further object is to provide a method for improving the viscosity indices of lubricating oils. Other objects and advantages of this invention will become apparent from the accompanying disclosure and discussion.

In accordance with this invention lubricating oil is treated with fluosulfonic acid to improve its viscosity index. This process is operated at temperatures within the range of about 10 to about 60° C., at about atmospheric pressure, and for a period of about 15 to about 120 minutes. If desired, a low-boiling hydrocarbon, such as iso- or normal pentane may be added to the lubricating oil-fluosulfonic acid mixture to aid in breaking the oil out of the acid, particularly when a large volume of acid is used. In commercial operation of this invention, the relative amounts of oil and acid used may vary considerably depending upon the extent of refining desired, however, it is generally preferred to use an acid to oil volume ratio in the range of about 0.5:1 to about 2:1.

A better understanding of my invention may be had by referring to the attached schematic flow diagram.

30 Into reactor 10, are introduced isopentane, lubricating oil, and fluosulfonic acid through lines 11, 12, and 13, respectively, where they are contacted for a period of about 15 to about 120 minutes at a temperature in the range of about 10 to about 60° C. and at sufficient pressure to maintain liquid phase. Effluent from reactor 10 is removed through line 14 to settler 15 where it is separated into two phases, an oil phase, and an acid phase. The oil phase is removed from settler 15 through line 16 to separation unit 17. In separation unit 17 isopentane, or whatever low-boiling hydrocarbon has been employed in the previous treatment, is removed through line 18 for recycle through line 11 to reactor 10. Hydrocarbons boiling below the initial boiling point of the untreated oil are removed through line 19. Lubricating oil is removed through line 20 and may be subjected to other treatment, as desired, such as being caustic washed and/or clay treated. In some instances, it may be desirable to caustic wash the oil phase before or at an intermediate point in the fractionation. Any heavier material is discharged through line 26. From settler 15, a fluosulfonic acid phase is removed through line 21. A portion may be recycled through line 25.

and another portion may be passed through line 27 to recovery unit 22, where purified fluosulfonic acid is recovered and passed through line 23 for recycle to reactor 10 through line 13. Any desired portion of the acid layer from settler 15 may be discarded through the outlet on line 21. Sludge and other materials are removed from acid recovery unit 22 through line 24.

To further illustrate some of the many aspects of this invention, the following specific example is given.

In three separate runs, a mixed-base lubricating oil, diluted with isopentane was treated with hydrofluoric acid, sulfuric acid, and fluosulfonic acid at about room temperature for a period of 60 minutes. (Addition of the fluosulfonic acid to the lubricating oil-isopentane mixture produced some temperature rise.) The volume ratio of oil to acid to isopentane was about 1:1:1. The acid and oil layers were separated and the oil caustic washed and topped to the initial boiling point of the untreated oil in a vacuum fractionating column to remove light ends.

The following physical data were determined for the product oils:

| Run                            |       | 1     | 2                              | 3                  |
|--------------------------------|-------|-------|--------------------------------|--------------------|
| Treating Agent                 | None  | HF    | H <sub>2</sub> SO <sub>4</sub> | HSO <sub>3</sub> F |
| Viscosity 100° F. SUS          | 388.3 | 374.9 | 346.0                          | 369.1              |
| Viscosity 210° F. SUS          | 55.52 | 55.17 | 54.62                          | 55.72              |
| Viscosity Index (Dean & Davis) | 85    | 87    | 95                             | 100                |
| API Gravity                    | 24.4  | 28.6  | 30.1                           | 30.0               |

From a comparison of the data from run 3, which represents the treatment of lubricating oil with fluosulfonic acid, with the data from runs 1 and 2, it may be seen that the fluosulfonic acid treatment of lubricating oil is superior to that of hydrofluoric acid or sulfuric acid, in that the viscosity index is increased by 15 points, from 85 of the original oil to 100.

Although this invention has been described and exemplified in terms of its preferred modifications, it is understood that various changes may be made without departing from the spirit of the process as disclosed and expressed in the claims.

I claim:

1. A process for refining a lubricating oil to improve its viscosity index, which comprises treating a lubricating oil with fluosulfonic acid

in the presence of a low-boiling hydrocarbon for a period of about 15 to about 120 minutes, at a temperature in the range of about 10 to about 60° C. and at sufficient pressure to maintain liquid phase, using a volume ratio of said fluosulfonic acid to oil about 0.5:1 to 2:1, separating said oil-acid-low-boiling hydrocarbon mixture into an oil phase and a fluosulfonic acid phase, and recovering from said lubricating oil phase a lubricating oil of improved viscosity index as a product of the process.

2. A process for refining a lubricating oil to improve its viscosity index, which comprises treating a lubricating oil with fluosulfonic acid as the only treating agent in the presence of a low-boiling hydrocarbon, separating said oil-acid-low-boiling hydrocarbon mixture into an oil phase and a fluosulfonic acid phase, and recovering a lubricating oil of improved viscosity index as a product of the process;

3. A process for improving a lubricating oil which comprises treating a lubricating oil with fluosulfonic acid as the only treating agent in the presence of a low-boiling hydrocarbon, recovering an improved lubricating oil as a product of the process.

4. A process for refining a lubricating oil to improve its viscosity index, which comprises treating a lubricating oil with fluosulfonic acid for a period of about 15 to about 120 minutes, at a temperature in the range of about 10 to about 60° C. and at sufficient pressure to maintain liquid phase, using a volume ratio of said fluosulfonic acid to oil about 0.5:1 to 2:1, separating said oil-acid mixture into an oil phase and a fluosulfonic acid phase, and recovering from said lubricating oil phase a lubricating oil of improved viscosity index as a product of the process.

PAUL H. CARNELL.

#### REFERENCES CITED

The following references are of record in the file of this patent:

#### UNITED STATES PATENTS

| Number    | Name     | Date          |
|-----------|----------|---------------|
| 1,950,878 | Burk     | Mar. 13, 1934 |
| 2,375,675 | Matuszak | May 8, 1945   |
| 2,378,762 | Frey     | June 19, 1945 |
| 2,428,753 | Linn     | Oct. 7, 1947  |